

Aug. 30, 1949.

K. SCHWARTZWALDER ET AL

**2,480,166**

## RESISTOR FOR THERMOGAUGES

Filed Jan. 8, 1945



*Sig. I*



Fig. 2



Fig. 3

## Inventors

*Karl Schwartzwalder,  
Alexander S. Pulka &  
Robert W. Smith,*

By Robert W. Smith  
Blackwelder, Spencer & Smith Attorneys

## UNITED STATES PATENT OFFICE

2,480,166

## RESISTOR FOR THERMOGAUGES

Karl Schwartzwalder, Holly, and Alexander S. Rulka and Robert W. Smith, Flint, Mich., assignors to General Motors Corporation, Detroit, Mich., a corporation of Delaware

Application January 8, 1945, Serial No. 571,812

5 Claims. (Cl. 201—76)

1

This invention relates generally to a thermogauge or temperature indicator and more particularly to the composition and manufacture of an improved resistor which varies in resistance or electric conductivity with temperature changes to operate an indicating instrument such as a differential galvanometer.

Although shown herein as employed in an indicator system for the temperature of the water cooling system of the internal combustion engine of an automotive vehicle, it will be apparent that the resistor is adapted for use in other types of temperature indicator systems or any electrical circuits wherein a predetermined variation in electric conductivity is desired in response to temperature changes.

According to the present invention, the resistor is in the nature of a ceramic oxide which may be composed primarily of magnetite and ferric oxide in combination with glass phase that acts as a fired bond.

The preferred composition with certain modifications thereof and the method of manufacturing the resistor to be described hereinafter have been found to produce a resistor which satisfies such desired physical requirements as a relatively large and substantially uniform temperature coefficient of resistance, electrical and chemical stability, no appreciable change in resistance on changes in applied voltage, a relatively low resistivity to minimize self-heating, and no directional effects in electrical conductivity in the range of voltages and currents encountered in practice.

In the drawings:

Figure 1 is a diagrammatic view of a part of an automobile showing an engine temperature indicator system.

Figure 2 is an enlarged sectional view showing the mounting of the resistor of the present invention.

Figure 3 is a perspective view of the resistor. Referring first to Figure 1, there has been shown a part of a conventional automotive vehicle including the usual body 4 with the windshield 6, the hood 8, and the instrument panel 10. The engine block 12 is provided with the head 14 in which is installed a thermostatic unit 16 for mounting the resistor of the present invention which is connected by the conductor 18 to a temperature indicator 20 such as a differential galvanometer of known type which may be connected in accordance with conventional practice through the ignition switch 22 to the

2

battery 24 having a ground connection 26 to the vehicle frame.

As shown in Figure 2, the unit 16 includes an adapter shell 28 which is threaded into an opening in a wall of the engine head 14 and supports an inwardly extending metal sleeve 30 having a closed inner end 32 and an open outer end with a flange 34 to engage the shell 28. The resistor 36, which may be in the form of a rod having flattened sides as shown in Figure 3, is mounted within the sleeve 30 with a spring 38 engaging the outer end of the resistor and holding the inner end of the resistor in contact with the sleeve end 32. Both the spring 38 and sides 10 of the resistor 36 are insulated from the sleeve 30 by means of insulation 40 such as fish paper.

The spring 38 is interposed between the outer end of the resistor 36 and the inner end of a contact stud 42 which is threaded at its outer 20 end to receive securing means such as the nuts 44 for the end of the conductor 18. The stud 42 is insulated from the adapter shell 28 and the flange 34 of sleeve 30 by means of washers 46 and 48 of Bakelite or similar insulating material and a sealing gasket 50 of rubber or the like. The outer washer 48 may be pressed over a knurled portion of the stud into contact with a shoulder 52 on the stud and the several parts of the unit 16 may be held together by turning over a flange 54 at the outer end of the shell 28 in the manner shown in Figure 2.

From the foregoing description it will be seen that one end of the resistor 36 will be grounded through the shell 30 and adapter 28 to the engine head 14 whereas the opposite end of the resistor is electrically connected through the spring 38, stud 42 and conductor 18 to the indicator 20. The heat from the water cooling system of the engine will be transmitted through the shell 30 to the resistor 36 which, as will be described hereinafter, has the characteristic of changing its electrical conductivity with a change in temperature, and the differential galvanometer 20 will be calibrated, as known in the art, to indicate the temperature of the water cooling system in response to the amount of current flow.

Referring now to the composition of the resistor 36 and the manufacture thereof which is the subject matter of the present invention, the resistor consists generally of a ceramic oxide composed primarily of magnetite and ferric oxide in combination with glass phase that acts as a fired bond. The composition which has been found to be most suitable for the use described hereabove 50 consists of approximately 71.1% of magnetite

( $\text{Fe}_3\text{O}_4$ ), 8.9% of ferric oxide ( $\text{Fe}_2\text{O}_3$ ), 10% borosilicate glass, and 10% magnesium borate glass.

In the foregoing composition the borosilicate glass may be that known as Pyrex and the magnesium borate glass may be made from 95%  $\text{B}_2\text{O}_3$  and 5%  $\text{MgO}$ , but it should be understood that the glasses can vary considerably in composition and the invention is not limited to use of these particular compositions.

It has also been found through actual practice that the preferred composition specified above can be varied as to both glass content and magnetite and ferric oxide contents. Addition of other metallic oxides such as chrome oxide, manganese oxide, nickel oxide, etc., have been made but for the present purpose, the above composition has thus far been the most suitable. In all cases some glass as a bond has been found to be desirable.

In the manufacture of the resistor, the constituents are first milled together for about one-half hour, preferably in a porcelain lined mill with porcelain balls. Then about 8% of a binder such as Dritex, which is a hydrogenated oil, is added and the mixture ground for about fifteen minutes.

The mixture is then removed from the mill, admixed with water, and granulated through a 20-mesh screen. It is dried in a steam drier and preferably again granulated through a further screen such as 14-mesh since when passed through the 20-mesh screen in a wet condition the length of some parts may be greater than 20-mesh and the mixture also swells to some extent after being pressed through this first screen.

The granulated mixture is then pressed in metal dies into the desired shape and form, such as the rod of Figure 3, and placed in a furnace at a temperature of about 700° F. for thirty minutes to burn out the Dritex. It has been found desirable to put the formed rods into stainless steel trays covered with calcined alumina during this heating operation and the alumina cleaned from the rod surface after cooling. The rods are then heated in a nitrogen atmosphere to about 1600° F. in a continuous belt type furnace on a forty-three minute cycle to melt the glasses and bond the materials together.

The ends of the rods are coated with copper, as indicated at 56 in Figure 3, in any known manner such as by spraying, and the resistance checked at 200° F. The rods may then be copper sprayed or coated in some other known manner to give the resistance desired for the particular application. In the present instance the resistor is formed into a strong, hard and relatively non-porous rod about one inch long and one-quarter inch in diameter which has the following properties.

Its resistivity at 25° C. is approximately 27 ohm-cm and its temperature coefficient of resistance is 3% per degree centigrade. This low resistivity minimizes self-heating and allows the resistor to carry higher currents without excessive self-heating. The resistor is chemically stable and unaffected by contact with ethylene glycol, alcohol, oil or grease. It is slightly soluble in water and must be protected when used under conditions of high humidity or where there is danger of contact with water or steam. For applications, however, where it is not feasible or desirable to avoid contact with water it appears from preliminary experiments that the elimina-

tion of the magnesium borate glass and use of only Pyrex as the glass phase in our composition may provide a resistor whose stability is not affected by humidity.

5 The electro-resistive effect is almost entirely absent in this resistor over the range of voltages encountered in practice, and for the range relevant to the present application, such as from 4 to 24 volts the change of resistance with voltage is negligible. The electrical conductivity also exhibits no directional effects in the range of voltages and currents encountered in practice and the resistor may be used in D. C. or A. C. circuits interchangeably without special precautions because of volume rectification effects. Since the resistor is formed in a slightly oxidizing atmosphere at a temperature much higher than that encountered over its operating range, it is electrically stable and requires no pre-aging or protection from direct contact with air or other oxidizing atmospheres.

10 It will be apparent that certain variations from the preferred method of manufacture described herein may be made by those skilled in the art, as well as modifications in the composition of the resistor, within the scope of the present invention as defined in the appended claims.

We claim:

15 30 1. A thermally sensitive resistor consisting of approximately 70% magnetite, 10% ferric oxide, and the remainder glass phase.

2. A thermally sensitive resistor consisting of approximately 70% magnetite, 10% ferric oxide, and a glass bond consisting of approximately equal amounts of borosilicate glass and magnesium borate glass.

3. A thermally sensitive resistor consisting of a bonded mixture of 71.1% magnetite, 8.9% ferric oxide, 10% borosilicate glass and 10% magnesium borate glass.

4. A thermally sensitive resistor comprising a glass bonded composition consisting of at least about 70% magnetite with a glass phase including magnesium borate glass.

5. A thermally sensitive resistor comprising a glass bonded composition having a substantially uniform temperature coefficient of resistance consisting of at least about 70% magnetite with a glass phase including borate glass.

KARL SCHWARTZWALDER.

ALEXANDER S. RULKA.

ROBERT W. SMITH.

#### REFERENCES CITED

The following references are of record in the file of this patent:

#### UNITED STATES PATENTS

| Number    | Name                  | Date          |
|-----------|-----------------------|---------------|
| 860,997   | Steinmetz             | July 23, 1907 |
| 2,027,413 | Andres                | Jan. 14, 1936 |
| 2,106,578 | Schwartzwalder et al. | Jan. 25, 1938 |
| 2,152,286 | Schoenmaker           | Mar. 28, 1939 |

#### FOREIGN PATENTS

| Number  | Country     | Date         |
|---------|-------------|--------------|
| 231,335 | Switzerland | June 1, 1944 |

#### OTHER REFERENCES

70 Ser. No. 377,578, Biefield (A. P. C.), pub. May 18, 1943.